

## 1

3,113,824

## DYEING WITH SULFUR DYES

Christoph Kohl, Frankfurt am Main, and Karl Schütz, Hubert Poppe, and Erwin Krüsche, Frankfurt am Main, Fechenheim, Germany, assignors to Cassella Farbwerke Mainkur Aktiengesellschaft, Frankfurt am Main, Fechenheim, Germany, a company of Germany  
No Drawing. Filed Feb. 24, 1960, Ser. No. 10,563  
Claims priority, application Germany Feb. 28, 1959  
6 Claims. (Cl. 8—37)

The present invention relates to a dyeing process. More particularly, the present invention relates to a new process for dyeing cellulose materials, such as native and regenerated cellulose, with sulfur dyes in the form of their water-soluble thiosulfonic acids together with alkali metal hydrogensulfides or sulfhydrides as reducing agents.

It is known that the commercial water-insoluble sulfur dyes are usually vatted with sodium sulfide, then brought from the strongly alkaline solutions onto the cellulose fiber in the form of their leuco compounds and finally oxidized on the fiber to form an insoluble dye. Sodium sulfide is preferably used because it is a cheap reducing agent and it also guarantees in practice a good solubility of all of the sulfur dyes. The application of sodium sulfide, however, involves a number of disadvantages which are due to the great alkalinity of the dye liquors containing same. Thus, it is known, for instance, that such dye-liquors affect unfavorably the softness and the feel of the dyed material. This concerns especially the regenerated cellulose. As, moreover, this fiber swells strongly during the dyeing process in alkaline dye liquors, a long and repeated rinsing becomes necessary afterwards, in order to remove completely the adhering dye liquor and the non-fixed dyestuff particles. Furthermore, difficulties arise frequently when unwinding the dyed bobbins because the fiber material to be dyed is liable to become sticky due to its strong swelling during the dyeing process.

For these reasons, efforts have been made for a long time to find a reducing agent of a reduced alkalinity which might be suited for the dyeing with sulfur dyes. Thus, a formaldehyde sodium sulfoxylate was recommended to be used in soda-alkaline solution for the purpose mentioned above. But quite apart from the fact that this reducing agent is much more expensive than sodium sulfide, it fails in many cases because of the inadequate solubility of numerous sulfur dyes in baths containing soda and formaldehyde sodium sulfoxylate. Furthermore, when working with formaldehyde sodium sulfoxylate, difficulties arise with regard to the reproducibility of shades due to over-reduction of the used dyes.

Attempts have also been made to use sodium hydrogen-sulfide or sulfhydride ( $\text{NaHS}$ ) instead of sodium sulfide ( $\text{Na}_2\text{S}$ ), which is as cheap as sodium sulfide when dyeing with sulfur dyes, because of its comparatively low alkalinity. However, it turned out that only a small fraction of the commercial water-insoluble sulfur dyes are sufficiently soluble in sodium sulfhydride. In the majority of cases, undesirable precipitates of the insoluble dye are formed in the dye liquors containing sodium sulfhydride. These precipitates lead to useless dyeings. Therefore, sodium sulfhydride could not gain ground, especially since commercial dyeing operations are carried out generally with mixtures of two or more different sulfur dyes and since sodium sulfhydride provides only a few possibilities of combination because of its narrow and limited applicability.

It has now been found that the water-soluble thiosulfonic acids of sulfur dyes which may be obtained for instance according to the process described in German Patents No. 88,392 and 91,720 and which have hitherto been used successfully in dyeing operations with sodium sulfide, can be excellently dyed with alkali-metal sulfhy-

## 2

drates as reducing agents, such as sodium sulfhydride, possibly by addition of soda.

This result could not be foreseen, for on the one hand there was the possibility that the alkalinity of the sodium sulfhydride would not suffice to split off the water-solubilizing thiosulfonic acid residues and that thus a fixation of the dye-stuff in its water-insoluble form could not take place. On the other hand, it was to be feared that even if the thiosulfonic acid residues had been split off, the same unfavorable conditions would appear, as it is the case when using water-insoluble sulfur dyes in a bath of sodium sulfhydride, i.e., that the undesired precipitation of undissolved dye would occur within the dye liquor.

It is surprising that the disadvantages mentioned above do not occur in the process of the present invention. It gives therefore, the possibility to use the water-soluble sulfur dye derivatives which yield very level dyeings and which are therefore already preferably employed in a simple dyeing method that guarantees the optimum save in the treatment of the material to be dyed.

The following Examples of the method of the present invention are given as illustrative only, the parts being by weight and all temperatures in degrees centigrade, the invention, however, not being limited to the specific details of the examples. References to "Col. Index" numbers refer to the "Colour Index of the Society of Dyers and Colourists," Second Edition, published by the said society at London in 1958.

## Example 1

80 grams of the thiosulfonic acid which has been prepared from Immedialbraun BR (Col. Index, vol. 3, p. 3449, No. 53,270) according to the process described in German Patent No. 91,720, are dissolved in water by short boiling and then this dye solution is diluted up to 20 liters. After addition of 120 cc. of a 22% sodium sulfhydride solution and 400 grams calcined Glauber's salt, 1 kg. spun viscose rayon is dyed in this solution during 1 hour at a temperature of 80–90°, subsequently rinsed and oxidized. The dyeing thus obtained corresponds in its depth of color and in its shade to the dyeing obtained by using sodium sulfide as reducing agent. The dyed material possesses an excellent feel.

## Example 2

50 grams of the thiosulfonic acid which has been prepared from Immedialbordo B (Col. Index, vol. 3, p. 3458, No. 53,721) according to the process described in German Patent No. 91,720, are dissolved in water by short boiling and the dyestuff solution is diluted up to 20 liters. After addition of 60 cc. of a 22% solution of sodium sulfhydride and 200 grams calcined Glauber's salt 1 kg. of spun viscose rayon is dyed at 50–60° during 1 hour, then rinsed and oxidized. The dyeing is about 10% more intense than that which may be obtained with the same quantity of dye when using sodium sulfide. Their shades are identical. The material thus dyed has a full and soft feel.

## Example 3

100 grams of the thiosulfonic acid which has been prepared from Immedialechbraun GGL (Col. Index, vol. 3, p. 3451, No. 53,327) according to the process described in German Patent No. 91,720 are dissolved in water by short boiling and the dye solution diluted up to 20 liters. After addition of 80 grams calcined soda, 200 cc. of a 22% solution of sodium sulfhydride and 400 g. calcined Glauber's salt 1 kg. cotton is dyed in this solution at 80–90° during 1 hour, then rinsed and oxidized. The dyeing is as intense as that which is obtained in a sodium sulfide bath on analogous conditions. However, the cotton dyed according to the present invention has a remarkably softer feel than the material dyed from the sodium sulfide bath.

It will be understood that this invention is susceptible to further modification and, accordingly, it is desired to comprehend such modifications within this invention as may fall within the scope of the appended claims.

We therefore, particularly point out and distinctly claim as our invention:

1. A process for dyeing a cellulosic material with a water-soluble thiosulfonic acid of a sulfur dye by treating the material to be dyed at an elevated temperature with a dye bath consisting essentially of the water-soluble thiosulfonic acid of the sulfur dye, an alkali-metal sulfhydride as a reducing agent, and water, and finishing the dyed material by rinsing, oxidizing and finally rinsing.

2. A process for dyeing a cellulosic material with a water-soluble thiosulfonic acid of a sulfur dye by treating the material to be dyed at an elevated temperature with a dye bath consisting essentially of the water-soluble thiosulfonic acid of the sulfur dye, sodium sulfhydride as a reducing agent, and water, and finishing the dyed material by rinsing, oxidizing and finally rinsing.

3. A cellulose material dyed with a sulfur dye by treating the material to be dyed at an elevated temperature

with a dye bath consisting essentially of the water-soluble thiosulfonic acid of the sulfur dye, alkali-metal sulfhydride as a reducing agent, and water, and finishing the dyed material by rinsing, oxidizing and finally rinsing.

4. A dye bath consisting essentially of a water-soluble thiosulfonic acid of a sulfur dye, an alkali-metal sulfhydride, and water.

5. A dye bath consisting essentially of a water-soluble thiosulfonic acid of a sulfur dye, an alkali-metal sulfhydride, soda, and water.

6. A dye bath consisting essentially of a water-soluble thiosulfonic acid of a sulfur dye, sodium sulfhydride, soda, and water.

15 References Cited in the file of this patent

UNITED STATES PATENTS

2,091,417 Schick et al. ----- Aug. 31, 1937

FOREIGN PATENTS

20 12,327 Great Britain ----- 1901  
88,392 Germany ----- Aug. 26, 1896  
91,720 Germany ----- March 29, 1897